

# United States Patent

[11] 3,610,311

[72] Inventor **Frank Holmes Simons**  
Charlotte, N.C.  
[21] Appl. No. **827,992**  
[22] Filed **May 26, 1969**  
[45] Patented **Oct. 5, 1971**  
[73] Assignee **Fiber Industries, Inc.**

2,349,290 5/1944 Loughborough ..... 57/153  
2,663,989 12/1953 Schlatter et al. ..... 57/153  
2,691,614 10/1954 Wilson ..... 57/153  
2,922,727 1/1960 Levison ..... 57/153  
2,955,345 10/1960 Howe ..... 28/75 R  
3,225,534 12/1965 Knospe ..... 57/157 S

[54] **TIRE YARN METHOD**  
**25 Claims, No Drawings**

*Primary Examiner*—Donald E. Watkins  
*Attorneys*—Thomas J. Morgan, Stephen D. Murphy and Louis Gubinsky

[52] U.S. Cl. .... **152/359,**  
57/153, 57/164, 117/138.8

[51] Int. Cl. .... **D02g 3/48,**  
**D02g 3/36**

[50] **Field of Search** .... **57/153, 140**  
**C, 164, 157 S; 28/75 R, 76 R; 117/138.8; 152/359**

[56] **References Cited**  
UNITED STATES PATENTS

3,475,204 10/1969 Patterson ..... 152/359 X

**ABSTRACT:** A method for reducing the strength loss and increasing hot elongation tolerance before break of a nylon tire cord which is subjected to an application of coating material during a hot stretching process, by applying to the tire cord a protective finish comprising an alkali metal soap of a fatty acid and an alkanolamine, particularly a lower trialkanolamine.

## TIRE YARN METHOD

## BACKGROUND

The present invention relates to improving the properties of nylon tire yarn and more particularly to reducing the susceptibility of nylon tire yarns to strength loss and poor hot stretch tolerance before break on the application of adhesive formulations used to improve the adhesive properties of the yarn to rubber during or prior to defined hot stretching operations.

Nylon tire yarns, particularly nylon 6,6, which is polyhexamethylene adipamide; nylon 6, which is polycaprolactam; and the like nylon tire cord materials including mixtures thereof are commonly subjected to an application of coating material to improve the adhesive qualities of the yarn to rubber. A common method of application is to dip the yarn into the adhesive material, such as a resorcinol-formaldehyde-latex or the like adhesive materials, and to subsequently hot stretch and simultaneously cure and dry the adhesive on the yarn. The temperature of the adhesive material as applied is generally that of the ambient temperature but the drying temperature during the hot stretching operation is sufficiently high so as to detrimentally affect the strength of the yarn unless it is protected from the heat, steam, pH changes and the like physical and chemical conditions existing during simultaneous drying-hot stretching procedures. While numerous yarn finishes are known in the art, finishes previously applied to reduce static electricity, increase yarn handling characteristics, i.e. reduce friction and the like, do not afford sufficient protection to the yarn when in the form of a twisted cord from the extreme conditions of an adhesive dip-hot stretch combination, which conditions reduce the physical properties of the yarn as hereinbefore described, particularly when the adhesive material is not dried prior to hot stretching.

It is therefore an object of the present invention to provide a nylon tire cord finish which reduces or eliminates strength loss and reduced stretch potential under elevated temperature conditions prior to break and other physical degradation of nylon tire cords occurring in the application of a finish during or prior to a cord hot stretching operation. It is another object of the present invention to provide a yarn finish which is easily and readily applied to the tire yarn, which finish decreases the yarn sensitivity to pH conditions during drying of adhesive material during a hot stretching operation. These and other objects will become apparent to those skilled in the art from the description of the invention which follows.

## THE INVENTION

In accordance with the invention, a method is provided for reducing the strength loss and brittle tendencies of nylon tire cord on being subjected to an application of adhesive during a hot stretching operation comprising forming a nylon multifilament cord having a tenacity of at least 6 grams per denier and a denier per filament of about 3 to 15 or higher i.e. 100 or more, applying an aqueous mixture of an alkali metal fatty acid soap and an alkanolamine to said cord and subsequently subjecting said cord to an adhesive application-hot stretching operation. The invention is particularly useful with nylon 6,6 wherein the applied alkali metal fatty acid soap is used with triethanolamine.

The present invention has been found to greatly reduce and even eliminate strength reduction and poor extensibility previously associated with an adhesive formulation dip-hot stretching operation in the formation of tire cords. While the exact theory of the present invention is not fully understood, it is believed that the alkaline nature of the finish composition protects the pH sensitive nylon from the degrading influence finishes commonly applied to such tire cords. Further, the finish apparently shields the cords from excessive penetration of the hot resinous material, thereby preventing excessive degradation of the nylon due to the deorientation of the fibers at the elevated temperatures and/or other degrading factors associated with the hot stretching process.

## DETAILS OF THE INVENTION

The present invention utilizes an alkali metal soap of a fatty acid and an alkanolamine in admixture, preferably in the form of an aqueous solution. The percentage of each of the components can vary depending upon the mutual solubilities and compatibilities of the various ingredients. Additionally, concentrations desired can be varied in accordance with the amount of finish to be applied, the viscosity of the finish com-

10 position, speed of application and the like considerations. As a general rule, it has been found that it is desirable to maintain the alkanolamine in a relatively high concentration, proportional to the concentration of soap present, in the finish composition. The quantity of soap in the finish formulation can 15 vary from being about equal to the amount of amine to less than one-half, e.g. to about 25 percent, of the amine material. The remainder of the composition is desirably water. Of course, organic solvents can be used in place of water for nonaqueous finish formulations.

20 Typically, the finish composition, by weight, comprises about 30 to 95 percent amine, 5 to 70 percent alkali metal fatty acid soap, and 0 to 65 percent water, the proportions being adjusted to a total of 100 percent. More preferably, the 25 finish solution comprises 40 to 50 percent amine, 18 to 28 percent alkali metal soap of a fatty acid, and 28 to 38 percent water. A particularly preferred composition comprises 45 percent triethanolamine, 22 percent of the sodium soap of coconut oil and 33 percent water.

30 Any of a number of dispersion mediums may be employed in the application of the finish formulation. Most often, the alkanolamine is a liquid at the temperature of application with which a liquid or solid soap may be admixed in the disclosed concentrations with or without the addition of water as 35 described in the preferred embodiments of the invention. Where necessary or desired, of course, other inert solvent dispersion mediums such as lower alcohols such as methanol, ethanol and mixtures thereof, as well as suspension and/or emulsion formulations may be employed with equally good 40 results.

45 The finish formulation should be applied so as to give at least about a 0.5 percent by weight pickup, based on weight of uncoated yarn. Preferably, 1 to 10 percent pickup, and most preferably about 1 to 2 percent finish pickup is employed. The 50 temperature of the finish formulation of the invention during yarn application may vary widely. Where aqueous formulations are employed, temperature most often will be in the range of about 5° to 95° C., preferably below 40° C., and most preferably about ambient temperature, e.g. 20°-25° C.

55 The amine used in the present invention is preferably a lower alkanolamine and, more preferably, a lower tri-alkanolamine. The term "lower" is used herein to describe a carbon chain of one to six carbon atoms, inclusive. Thus, mono-, di-, and tri-alkanolamines are contemplated amines wherein each of the alkanol segments contains one to six carbon atoms. Typical amines include monomethanolamine, dimethanolamine, trimethanolamine, monoethanolamine, diethanolamine, triethanolamine, monopropanolamine, 60 dipropanolamine, tripropanolamine, monobutanolamine, dibutanolamine, tributanolamine, mixtures of the same and the like amines. Of course, di- and tri- substituted amines wherein the alkanol groups are dissimilar, i.e. methanol-diethanolamine, can also be used.

65 The fatty acid soaps utilized in the present invention are alkali metal soaps of fatty acid groups of 12 to 22 or more carbon atoms. The fatty acid groups can be obtained from any of the numerous sources of saponifiable fatty chains such as animal and vegetable oils, petroleum stocks and the like. Of 70 particular interest are the glyceride esters of fatty acids which are readily hydrolyzed, using an alkali metal hydroxide, to the corresponding alkali metal soap of a fatty acid. In such instance, it has been found to be particularly desirable to utilize the esterification product as such, without removal of the 75 formed glyceride.

In addition to having residual glycerides in the saponification product, vegetable and the like oils are normally a mixture of several different fatty acids of varying chain length and degree of unsaturation. In particular, the saturated or nondrying oils are recommended for use in the present invention, although drying and semidrying oils can also be used either as such or following hydrogenation. Typical animal, vegetable and marine oils of the type useful herein include soya, tung, linseed, coconut, menhaden, anchovy, tuna, oiticica, safflower, rape seed and the like. Thus, typical hydrogenated or saturated fatty acids include stearic, lauric, palmitic, behenic, myristic, arachidic, tridecanoic, pentadecanoic, heptadecanoic, nonadecanoic and the like. The preferred coconut oil generally contains caprylic, copric, lauric, myristic, palmitic, steric, oleic, linoleic and linolenic acids. The alkali metal used for the formation of the soap may be any of the group 1(a) alkali metal periodic chart elements and preferably is selected from lithium, sodium and potassium. Sodium and potassium are most preferred, particularly because of their availability, low cost and effectiveness. The alkali metal is mostly commonly utilized in the form of the corresponding hydroxide in the saponification of the fatty acid, or ester or other saponifiable derivative thereof.

The nylon yarn utilized in the present invention is normally considered to be a high-tenacity multifilament yarn. Thus, the yarn has a tenacity of at least 6 grams per denier and may have a tenacity as high as 10 grams per denier or more. Normally, the higher the tenacity, the better suited such material is for tire cord. The denier of individual filaments in such high-tenacity yarns is normally higher than that of textile grade nylon filaments, and preferably is in the range of about three to 15. Higher deniers could be used provided the desired yarn flexibility is retained. The number of filaments per cord can very greatly. However, it is preferred to have a large number of filaments such as more than 10, and more preferably more than 100 filaments per cord. A typical tire yarn commonly has about 140 filaments per cord.

The form of the coating material applied to the tire cord containing the finish described herein will vary depending upon the particular tire manufacturing operation involved. The present invention has particular utility in combination with adhesive application to the tire cord. The adhesive coating material is usually employed to enhance the adhesiveness of the cord to rubber, and thus, numerous materials are utilized. Such compositions can be aqueous solutions or emulsions as well as solvent solutions and/or suspensions. Similarly the particular type of adhesive used, the manufacturer's preference to employment with his particular integrated system and the like determine the particular condition in

turing processes involving the application of cold adhesive formulation to a plied or otherwise twisted cord, or fabric constructed therefrom, which is subsequently hot stretched before the adhesive has dried. Although the invention is exemplified with respect to this kind of process, it should be understood that yarn which may demonstrate similar undesired properties because of different reasons may also be protected and benefited by the present invention.

While the invention has been described more particularly with reference to tire cord, it is therefore to be recognized that the present invention is generally related to industrial yarns to which coating, particularly adhesive materials, are subsequently applied during hot stretching operations in a plied or twisted cord configuration. Thus, while the tire yarn is the biggest end use of such industrial yarns, conveyor belts, v-belts, drive belts, and the like, wherein resinous materials are applied to increase the adhesion to rubber or other materials are likewise within the scope of the present invention.

The invention will be more fully described by reference to the present examples. The following are examples which illustrate certain preferred embodiments of the present invention. Unless otherwise indicated, all temperatures are in degrees centigrade and all parts are by weight.

25

#### EXAMPLE I

An industrial nylon cord is formed by twisting a 840/140 nylon 6,6 multifilament yarn having a tenacity of 9.0 grams per denier and an elongation at the break of 15.5 percent, 12 turns in the "S" direction in the singles and then plying two such yarns by twisting them 12 turns in the "Z" direction. The cord has an average breaking strength of about 31.8 pounds and average elongation at the break of about 21.8 percent. All yarns contain a normal spin finish. The cord is then additionally topcoated as stated in table I utilizing an applicator roll procedure and, following drying of the coating material, is dipped in a standard resorcinol-formaldehyde-latex adhesive at room temperature and immediately passed before the adhesive dries through a 420° F. oven for 20 seconds while being stretched 12 percent. This stretching operation is referred to as "single pass processing." The term "topcoating" and the like refers to the additional soap-alkanolamine finish formulation which is applied to the yarn in addition to the normal spin finish.

In a like manner, industrial nylon cord may be hot stretched at a temperature within the range of about 300° F. up to the degradation and/or melting point of the polymer, preferably in the range of about 300° to 500° C., following application of the finish formulation of the invention.

50

TABLE I

| Sample | Top coat             | Denier | Greige cord               |                             |                               | Processed cord            |                               |                           | Pick-up on yarn (percent) |
|--------|----------------------|--------|---------------------------|-----------------------------|-------------------------------|---------------------------|-------------------------------|---------------------------|---------------------------|
|        |                      |        | Breaking strength (pound) | Tenacity (grams per denier) | Elongation at break (percent) | Breaking strength (pound) | Elongation at break (percent) | Breaking strength (pound) |                           |
| 1..... | None.....            | 1867   | 31.5                      | 7.65                        | 21.4                          | 30.9                      | 14.1                          | 30.9                      | 98                        |
| 2..... | Lubricating oil..... | 1899   | 32.2                      | 7.69                        | 23.9                          | 23.8                      | 11.0                          | 23.8                      | 74                        |
| 3..... | Ivory soap.....      | 1862   | 31.4                      | 7.67                        | 23.2                          | 31.7                      | 16.1                          | 31.7                      | 101                       |
| 4..... | Coconut soap.....    | 1898   | 32.4                      | 7.74                        | 20.7                          | 32.6                      | 15.6                          | 32.6                      | 101                       |
| 5..... | Coconut soap.....    | 1848   | 31.0                      | 7.61                        | 21.8                          | 31.2                      | 15.6                          | 31.2                      | 101                       |

which the adhesive material is applied to the cord. Also, the method of application can be varied. Application such as by brushing, spraying and the like can be used, with a dip application being normally preferred because of the speed and thoroughness of application thereby achieved.

As stated hereinbefore, the present invention, through the application of the soap-alkanolamine mixture to nylon yarn, prevents strength loss and the tendency to form comparatively brittle yarn segments resulting in a low tolerance to hot stretch as occurs during certain manufacturing operations. These adverse effects are particularly pronounced during the manufac-

70 This example illustrates enhanced strength retention, amounting to an actual slight increase in cord strength, resulting from the inclusion of a soap as disclosed herein in a topcoating formulation. It is also interesting to note that the control cord (Sample 1) loses relatively little strength under the single pass processing utilized in example I.

The viscosity of the topcoating formulation can very widely as long as ease of application is maintained with respect to the particular application technique and temperature employed. Thus, viscosity could correspond to that of mineral spirits up to that of heavy motor oil where desired. Preferably, viscosity

is regulated to be about that of water at the preferred temperature of application, which is room temperature, e.g. about 22° C., while a room temperature viscosity within the range of about 10-20 centipoises is highly preferred for high-speed yarn finishing. Although a number of exemplary oils have been stated hereinbefore for use with the invention, an oil having a relatively high saponification number is preferred since it will exhibit excellent miscibility and/or solubility with hydrophilic finish formulation components, i.e. water and triethanolamine, at room temperature. As the saponification number of the oil decreases, there is a proportional decrease in water solubility since the oil would be characterized by a lower number of available acid radicals per unit weight, saponification number being a measure of total free and combined acids, e.g. esters, expressed as number of milligrams of potassium hydroxide required for complete saponification of one gram of substance. To avoid the use of elevated temperatures during application and/or suspension agents, the oil employed, which can be a mixture of two or more oils as well as one or more pure acids, should have a saponification number over 200, and preferably over 250. The saponification number of coconut oil is within the range of about 254-262. Palm oil, depending upon geographical and extractive origin, can have a saponification number as low as 200 and as high as 255. As examples of oils having values slightly below the preferred values, there may be mentioned cottonseed oil and corn oil with saponification numbers within the ranges of 194-196 and 187-193, respectively. Of course, cottonseed, corn and similar oils are still usable with the invention but as saponification number decreases further, elevated temperatures are required.

The data in table II demonstrates the contribution of the alkanolamine to increase the cord's extensibility at elevated temperatures encountered during industrial processing, particularly during tire yarn manufacturing operations, and pinpoints preferred and optimum topcoat formulation ranges. It is interesting to note the relatively minor contribution required of the soap under the stretching conditions employed in example II (Compare to Sample 1 of example I). The use of a lubricating oil in place of the soap-triethanolamine finish yields about a 14 percent stretch-break under the conditions of example II.

Although the triethanolamine where used alone under the particular processing conditions of example II does not result in a material reduction in yarn breaking strength, the top-coated yarn will abrade to an unacceptable degree where subjected to normal friction encountered during many high-friction yarn processes, Such as high-speed twisting of the order of 6,000 rotations per minute onto a spindle through a balloon guide. Of course, in a sense, abrasion of the yarn surface also produces a final product of reduced tenacity. The alkali metal fatty acid soap is an acceptable yarn lubricant under normal high-speed yarn processing conditions and is therefore, included in the finish formulation of the invention for its lubricating properties in addition to its function as a yarn strength retention agent.

### EXAMPLE III

The nylon industrial cord of example I is processed in accordance with example I with the topcoating finish formulations as described in table III being applied prior to the adhesive application-hot stretch single pass process.

TABLE III

|                                         | Sample                        |                               |                               |                                        |                                              |
|-----------------------------------------|-------------------------------|-------------------------------|-------------------------------|----------------------------------------|----------------------------------------------|
|                                         | 13                            |                               | 14                            |                                        | 15                                           |
|                                         | Topcoat                       |                               | 16                            |                                        | 17                                           |
|                                         | 18% ivory<br>soap;<br>82% TEA | 18% ivory<br>soap;<br>82% TEA | 33% ivory<br>soap;<br>67% TEA | 23% coconut<br>sodium soap;<br>77% TEA | 33% coconut<br>potassium<br>soap;<br>67% TEA |
| Topcoat concentration in water, percent | 100                           | 43                            | 50                            | 100                                    | 50                                           |
| Application temperature, ° C            | 40                            | 22                            | 22                            | 40                                     | 22                                           |
| Greige cord:                            |                               |                               |                               |                                        |                                              |
| Denier                                  | 1,913                         | 1,872                         | 1,864                         | 1,928                                  | 1,859                                        |
| Breaking strength, lb                   | 31.5                          | 31.7                          | 32.2                          | 30.1                                   | 31.9                                         |
| Tenacity, g.p.d.                        | 7.47                          | 7.69                          | 7.83                          | 7.08                                   | 7.79                                         |
| Elongation at the break, percent        | 21.0                          | 22.8                          | 22.0                          | 21.2                                   | 21.5                                         |
| Processed cord:                         |                               |                               |                               |                                        |                                              |
| Stretch-break, percent                  | 24                            | 20                            | 20                            | 22                                     | 20                                           |
| Breaking strength, lb                   | 30.7                          | 32.6                          | 32.8                          | 30.4                                   | 32.2                                         |
| Elongation at the break, percent        | 15.9                          | 15.0                          | 13.8                          | 13.5                                   | 13.1                                         |
| Strength retention, percent             | 97                            | 103                           | 102                           | 101                                    | 101                                          |

TEA = Triethanolamine.

Ivory soap = A commercial bar soap of mixed oleates, stearates, and coconut oil.

<sup>1</sup> No water.

<sup>2</sup> Ambient.

### EXAMPLE II

The nylon industrial cord of example I is topcoated with a finish formulation containing varying amounts of coconut soap and triethanolamine as detailed in table II and is then subjected to the single pass processing described in example I.

With reference to the above examples, the Ivory soap employed is the commercially available material available from Proctor and Gamble of Cincinnati, Ohio.

Various modifications within the scope of the invention will appear obvious to those skilled in the art. For example, where desired only one of the finish formulation components may be

TABLE II.—EFFECT OF SOAP-TRIETHANOLAMINE RATIO ON STRETCH BREAK IN SINGLE PASS CORD PROCESSING

|                                    | Sample |      |      |      |      |      |      |
|------------------------------------|--------|------|------|------|------|------|------|
|                                    | 6      | 7    | 8    | 9    | 10   | 11   | 12   |
| Percent coconut soap in topcoat    | 0      | 23   | 33   | 50   | 67   | 100  |      |
| Percent triethanolamine in topcoat | 100    | 77   | 67   | 50   | 33   |      |      |
| Stretch-break, percent             | 18     | 18   | 18   | 16   | 14   | 15.2 | 14   |
| Breaking-strength (lb.)            | 31.6   | 31.4 | 31.8 | 31.2 | 31.7 | 32.6 | 29.0 |
| Elongation at break, percent       | 15.8   | 14.0 | 14.2 | 13.8 | 14.6 | 15.6 | 14.4 |

"Stretch-Break-Percent" as used in table II is a measurement of the cord's tolerance to a hot stretch before breaking at the temperature employed during cord processing (420° F. in example II)

employed since it is apparent that the soap is primarily involved with strength retention while the alkanolamine contributes chiefly to hot stretch tolerance.

What is claimed is:

1. A nylon multifilament yarn having a tenacity of at least 6 grams per denier, a denier per filament of about 3 to 15 and having substantially uniformly distributed thereon in an amount of at least 0.5 percent by weight of the yarn a topcoating consisting essentially of an alkali metal fatty acid soap wherein said soap is selected from the saponification products of fatty acid materials having fatty groups within the range of about 12 to 22 carbon atoms and the alkali metal is an element of group 1(a) of the periodic chart and a lower alkanolamine, said yarn being characterized by lack of strength loss and good tolerance to hot stretching during a coating-hot stretching operation.

2. The yarn of claim 1 in the form of a tire cord.

3. An article of manufacture comprising the yarn of claim 1 as a reinforcement material.

4. A tire reinforced with the cord of claim 2.

5. A process for preventing strength loss and reduced tolerance to hot stretching of nylon industrial monofilament or multifilament yarn during yarn processing which process comprises applying a finish formulation of a mixture of an alkali metal fatty acid soap wherein said soap is selected from the saponification products of fatty acid materials having fatty groups within the range of about 12 to 22 carbon atoms and the alkali metal is an element of group 1(a) of the periodic chart and a lower alkanolamine to said yarn to give a pickup of at least about 0.5 percent by weight of finish on the yarn prior to said yarn processing.

6. The process of claim 5 wherein said nylon is nylon 6,6.

7. The process of claim 5 wherein said soap is the saponification product of coconut oil.

8. The process of claim 5 wherein the saponification product is used without the separation of the glycerols formed during said saponification.

9. The process of claim 5 wherein said amine is a tri-alkanolamine.

10. The process of claim 9 wherein said amine is triethanolamine.

11. The process of claim 5 wherein said soap and said alkanolamine are in the ratio of soap/amine in the finish formulation of about 1/1 to 1/4 by weight.

12. The process of claim 5 wherein said finish formulation, per 100 parts, contains 30-95 parts of said amine, 5-70 parts of said soap and 0-65 parts water, by weight.

13. The process of claim 9 wherein said finish formulation, per 100 parts, contains 40-50 parts of said amine, 18-28 parts of said soap and 28-38 parts  $H_2O$ , by weight.

14. The process of claim 10 wherein said finish formulation, per 100 parts, by weight contains about 45 parts of said amine, about 22 parts of said soap, said soap being coconut soap, and about 33 parts water.

15. A process for producing a nylon tire cord which com-

prises preparing a nylon multifilament yarn having a tenacity of at least about 6 grams per denier and a denier per filament of about 3 to 15; topcoating said yarn with a lower alkanolamine to give a pickup of at least about 0.5 percent by weight of said amine on said yarn; forming a twisted cord from said yarn; applying a resorcinol-formaldehyde-latex adhesive to said cord and hot stretching said cord before said adhesive dries to simultaneously cure and dry said adhesive on said yarn during said hot stretching.

16. The process of claim 15 wherein said alkanolamine is triethanolamine.

17. A process for coating and hot stretching nylon industrial monofilament or multifilament yarn while reducing strength loss and increasing tolerance to hot stretching of said yarn during said coating-hot stretching operation which comprises forming a nylon yarn having a tenacity of at least 6 grams per denier and a denier per filament of at least about 3 to 15; applying a finish formulation of a mixture of an alkali metal fatty acid soap wherein said soap is selected from the saponification

products of fatty acid materials having fatty groups within the range of about 12 to 22 carbon atoms and the alkali metal is an element of group 1(a) of the periodic chart and lower alkanolamine to said yarn to give a pickup of at least 0.5 percent by weight of finish on the yarn and subsequently subjecting said yarn to a coating-hot stretching operation.

18. The process of claim 17 wherein said yarn is a multifilament yarn twisted and subjected to a coating-hot stretching operation to form a tire cord.

19. The process of claim 18 wherein said coating-hot stretching operation comprises the application of an adhesive formulation to said cord and hot stretching of said cord before said adhesive formulation dries.

20. The process of claim 19 wherein said soap is the saponification product of coconut oil and said amine is triethanolamine.

21. The process of claim 19 wherein said soap and said alkanolamine are in the ratio of soap/amine in the finish formulation of about 1/1 to 1/4 by weight.

22. The process of claim 19 wherein said finish formulation, per 100 parts, contains 30-95 parts of said amine, 5-70 parts of said soap and 0-65 parts water, by weight.

23. The process of claim 19 wherein said finish formulation, per 100 parts, contains 40-50 parts of said amine, 18-28 parts of said soap and 28-38 parts  $H_2O$ , by weight.

24. The process of claim 19 wherein said finish formulation, per 100 parts, by weight contains about 45 parts of said amine, about 22 parts of said soap, said soap being coconut soap, and about 33 parts water.

25. The process of claim 24 wherein said coating is a resorcinol-formaldehyde-latex adhesive.